

## UNITED STATES PATENT OFFICE

2,172,023

## HEAT-RESISTANT ALLOY

John D. Gat, Pittsburgh, Pa.

No Drawing. Application August 30, 1937,  
Serial No. 161,680

2 Claims. (CL. 75—124)

This invention relates to heat resistant alloys and, more particularly, to a heat resistant alloy containing aluminum.

One object of this invention is to provide an improved heat resistant alloy which is substantially free from carbides at its grain boundaries.

Another object of this invention is to provide a heat resistant alloy having hot-working characteristics comparable to the more expensive alloys of the stainless type.

A further object is to provide an inexpensive alloy having improved electrical resistance properties at elevated temperatures.

The value of aluminum additions to steel to prevent oxidation at elevated temperatures has long been recognized and discussed, but aluminum additions cause excessive grain growth which prevents its being satisfactorily hot or cold-worked. This is attributed to the fact that, upon cooling, the carbon present in iron-aluminum alloys, segregates at the grain boundaries and forms a brittle, hard film of complex carbides which surround the iron-aluminum grains. This film causes brittleness and quick failure, due to rapid deterioration of such carbides. Increasing amounts of carbon and aluminum naturally tend to aggravate brittleness and large grain structure.

Thus, carbon, even to the extent of only a few hundredths of one per cent., so affects the ductility of the iron-aluminum alloy as to prevent its being practically hot or cold reduced, as is so often desired. With the carbon content unchanged, but by increasing the percentage of aluminum present, such as from 5 to 15 per cent., the ductility becomes less while the ability to roll the metal becomes almost impossible. The total elimination of carbon might eliminate some of the above difficulties but such elimination places it outside the capabilities of present industrial furnaces. It is practically impossible to reduce, in present furnaces, the carbon content to within limits which would make it permissible to make iron-aluminum alloys free from carbide precipitations at the grain boundaries.

The present invention overcomes the above disadvantages in the manufacture of heat resistant alloys and produces an iron-aluminum alloy inherently more stable at elevated temperatures than the usual iron-aluminum alloys. Such an improved alloy is also ductile, machinable and weldable, due to the fine distribution and elimination of the deleterious carbides from the grain boundaries.

This is primarily accomplished by the pres-

ence of an element or elements which removes highly soluble carbides from between the grain boundaries by forming insoluble carbides which are so finely and uniformly distributed throughout the iron-aluminum mass that they have no deleterious effect on ductility or corrosion resistance of the metal. Such carbides have a low solubility at elevated temperatures and prevent any substantial amount of carbides at grain boundaries, even after repeated heating and cooling, which is common in the use of such heat resistant articles.

The elements to accomplish this purpose include primarily titanium; although molybdenum, tantalum, columbium or metals of similar characteristics may be utilized. Such an element as titanium, for example, is added to the metal in quantities defined by the carbon content so as to produce uniformly distributed, fine carbides of low solubility throughout the mass. Under this invention, the carbides are substantially eliminated from the grain boundaries of the alloy.

I have found that the amount of titanium, for example, should be about six (6) times the amount of carbon present. Thus, if the carbon is approximately 0.10 per cent. the titanium addition should be about six (6) times that amount or approximately 0.60 per cent. Thus, for example only, Table I indicates the approximate amounts of aluminum, titanium and carbon present in low carbon alloys having:

(A) High ductility at hot-working temperatures and relatively low physical properties at elevated temperatures (1600 degrees Fahrenheit), and

(B) High ductility at hot-working temperatures but relatively high physical properties at the same elevated temperatures, as follows:

Table I

|                 | A                           | B               |    |
|-----------------|-----------------------------|-----------------|----|
| Aluminum.....   | Over 6%.....                | Over 6%.....    | 45 |
| Titanium.....   | Less than 1%.....           | Over 1%.....    |    |
| Carbon.....     | 0.16% maximum.....          | Over 0.16%..... |    |
| Manganese.....  |                             |                 |    |
| Sulphur.....    | residuals not exceeding 2%. |                 |    |
| Phosphorus..... |                             |                 |    |
| Silicon.....    |                             |                 |    |
| Iron.....       | Remainder.....              | Remainder.....  | 50 |

While I have shown the amounts of titanium that should preferably be added in order to distribute the carbides uniformly so that the grain boundaries of the Fe-Al solid solution are sub-

stantially free therefrom, it is to be understood that I may use other elements for the same purpose. Thus, columbium may be used in amounts sufficient to distribute the carbides which, as some tests indicate, will approximate about eight (8) to nine (9) times the amount of carbon.

In addition to the above mentioned advantages of such an alloy, wide distribution of these insoluble carbides throughout and within the grains leads to more nuclei of crystallization which promotes an inherent fine grain structure, and increases stiffness proportional to the amount of carbides present which exhibits itself primarily as strength at elevated temperatures, where strength is needed. Stiffness produced by fine distribution of carbides, does not affect either ductility or workability of the metal either in its hot or cold state.

Such an alloy can be worked into thin sections providing inexpensive heating elements having improved electrical properties over the more expensive and more difficult to work chromium and chromium-nickel alloys commonly used for this purpose. This improvement manifests itself in a material increase of ohmic resistance expressed in microhms per cubic centimeter. Thus, for example, an alloy of my invention containing about 8 per cent. aluminum and 0.30 per cent. titanium has a resistance of 160 microhms per cubic centimeter, as compared to 132 microhms per cubic centimeter at the same

temperature for so-called "Nichrome" metal utilized especially for electric heating units.

While I have described one embodiment of the present invention, it is to be expressly understood that various modifications may be made in forming the heat resistant alloy in accordance with the scope of the appended claims.

I claim:

1. A ductile, heat-resistant iron-aluminum alloy including a carbon content not greater than 0.16 per cent., not less than 6 per cent. aluminum and sufficient titanium to prevent any substantial presence of carbides at the grain boundaries of the alloy, said titanium being approximately six (6) times the amount of carbon and at no time exceeding 1 per cent.; manganese, sulphur, phosphorus and silicon in combined amounts not to exceed 2 per cent., and the remainder being iron.

2. A ductile, heat-resistant alloy including a carbon content not greater than 0.16 per cent., not less than 6 per cent. of aluminum and with a sufficient member of the group consisting of titanium, molybdenum, tantalum and columbium to prevent any substantial presence of carbides at the grain boundaries of the alloy, said member being not greater than six (6) times the amount of carbon and at no time exceeding 1 per cent., manganese, sulphur, phosphorus and silicon in combined amounts not to exceed 2 per cent., and the remainder being iron.

JOHN D. GAT.